

1

2,990,368

**LUBRICATING GREASE COMPOSITIONS CONTAINING AN ALKYLAMINOCARBAZOLE**  
 Ralph B. Thompson, Hinsdale, Ill., assignor, by mesne assignments, to Universal Oil Products Company, Des Plaines, Ill., a corporation of Delaware  
 No Drawing. Filed May 9, 1958, Ser. No. 734,118  
 12 Claims. (Cl. 252—40.7)

This invention relates to the stabilization of synthetic grease and more particularly to a novel method of preventing and/or retarding deterioration thereof. The present application is a continuation-in-part of my earlier application Serial No. 537,539, filed September 29, 1955, now Patent No. 2,864,676.

Synthetic greases include lithium base grease, sodium base grease, potassium base grease, calcium base grease, barium base grease, strontium base grease, aluminum base grease, beryllium base grease, cadmium base grease, magnesium base grease, lead soap grease, complex soap grease, etc., or mixtures known as mixed base greases. These greases are solid or semi-solid gels and in general are prepared by the addition to mineral oils of hydrocarbon-soluble metal soaps or salts of higher fatty acids as, for example, lithium stearate, calcium stearate, aluminum naphthenate, etc. In another method, the metal soap or salt is added to synthetic oils including, for example, di-(2-ethylhexyl) sebacate or azelate, di-tetradecyl sebacate, tricresyl phosphate, polyalkylene oxides, silicones, alkyl or alkyl aryl polysiloxanes or blends of these with petroleum oil. The grease may contain thickening agents such as silica, carbon black, polyacrylates, talc, polyamides, alkylureas, etc. Another type of grease is prepared from oxidized petroleum wax to which the saponifiable base is combined with the proper amount of the desired saponifying agent, and the resultant mixture processed to produce a grease.

In one embodiment the present invention relates to a method of stabilizing synthetic grease which comprises incorporating therein a stabilizing concentration of an alkylaminocarbazole inhibitor.

In a specific embodiment the present invention relates to a method of stabilizing lithium base grease which comprises incorporating therein from about 0.0001% to about 5% by weight of 3-octylaminocarbazole.

In still another embodiment, the present invention relates to a synthetic grease containing a stabilizing concentration of the inhibitor herein set forth.

The stabilization of synthetic grease presents problems considerably different from those encountered in the stabilization of petroleum greases, for example. Synthetic greases have been developed for use at high temperatures and therefore require a stabilizing agent which will be effective at the high temperatures encountered during use of the synthetic grease. Furthermore, the chemical composition of synthetic greases is different from the chemical composition of petroleum greases, and these different properties accordingly present different problems.

In accordance with the present invention stabilization of synthetic grease is accomplished by incorporating therein an alkylaminocarbazole inhibitor. Illustrative inhibitors include 1-ethylaminocarbazole, 1-propylaminocarbazole, 1-butylaminocarbazole, 1-amylaminocarbazole, 1-hexylaminocarbazole, 1-heptylaminocarbazole, 1-octylaminocarbazole, 1-nonylaminocarbazole, 1-decylaminocarbazole, 1-undecylaminocarbazole, 1-dodecylaminocarbazole, etc., 3-ethylaminocarbazole, 3-propylaminocarbazole, 3-butylaminocarbazole, 3-amylaminocarbazole, 3-hexylaminocarbazole, 3-heptylaminocarbazole, 3-octylaminocarbazole, 3-nonylaminocarbazole, 3-decylaminocarbazole, 3-undecylaminocarbazole, 3-dodecylaminocarbazole, etc., 3,6-diethylaminocarbazole, 3,6-dipropylami-

2

nocarbazole, 3,6-dibutylaminocarbazole, 3,6-diamylaminocarbazole, 3,6-dihexylaminocarbazole, 3,6-dihexylaminocarbazole, 3,6-dioctylaminocarbazole, 3,6-dinonylaminocarbazole, 3,6-didecylaminocarbazole, 3,6-diundecylaminocarbazole, 3,6-didodecylaminocarbazole, etc., 1,3,6,8-tetraethylaminocarbazole, 1,3,6,8-tetrapropylamino carbazole, 1,3,6,8-tetrabutylaminocarbazole, 1,3,6,8-tetraamylaminocarbazole, 1,3,6,8-tetrahexylaminocarbazole, 1,3,6,8-tetraheptylaminocarbazole, 1,3,6,8-tetracetylaminocarbazole, etc. 2,3,6,7-tetraethylaminocarbazole, 2,3,6,7-aminocarbazole, 2,3,6,7-tetrapropylamino carbazole, 2,3,6,7-tetrabutylaminocarbazole, 2,3,6,7-tetrahexylaminocarbazole, 2,3,6,7-tetraoctylaminocarbazole, etc. It is understood that the specific compounds set forth above are illustrative and that corresponding compounds having the substitutions in other positions may be utilized.

In another embodiment, aminocarbazoles also having a substituent attached to the imino nitrogen may be used. The imino nitrogen is the heterocyclic nitrogen in the 5-membered ring. Illustrative examples of inhibitors in this class include N-ethyl-3-ethylaminocarbazole, N-ethyl-3-propylaminocarbazole, N-ethyl-3-butylaminocarbazole, N-ethyl-3-amylaminocarbazole, N-ethyl-3-hexylaminocarbazole, N-ethyl-3-octylaminocarbazole, etc., N-propyl-3-ethylaminocarbazole, N-propyl-3-butylaminocarbazole, N-propyl-3-hexylaminocarbazole, N-propyl-3-octylaminocarbazole, N-propyl-3-heptylaminocarbazole, N-propyl-3-heptylaminocarbazole, N-propyl-3-octylaminocarbazole, etc., N-butyl-3-ethylaminocarbazole, N-butyl-3-propylaminocarbazole, N-butyl-3-butylaminocarbazole, N-butyl-3-amylaminocarbazole, N-butyl-3-hexylaminocarbazole, N-butyl-3-octylaminocarbazole, N-butyl-3-heptylaminocarbazole, N-butyl-3-octylaminocarbazole, N-amyl-3-ethylaminocarbazole, N-amyl-3-butylaminocarbazole, N-amyl-3-hexylaminocarbazole, N-amyl-3-octylaminocarbazole, etc., N-hexyl-3-ethylaminocarbazole, N-hexyl-3-propylaminocarbazole, N-hexyl-3-butylaminocarbazole, N-hexyl-3-hexylaminocarbazole, N-hexyl-3-octylaminocarbazole, etc., N-ethyl-3,6,7-tetrapropylamino carbazole, N-ethyl-2,3,6,7-tetrabutylaminocarbazole, N-ethyl-2,3,6,7-tetrahexylaminocarbazole, etc., N-propyl-2,3,6,7-tetraethylaminocarbazole, N-propyl-2,3,6,7-tetrapropylamino carbazole, N-propyl-2,3,6,7-tetrabutylaminocarbazole, N-propyl-2,3,6,7-tetrahexylaminocarbazole, etc., N-propyl-1,3,6,8-tetrabutylaminocarbazole, etc. Here again, it is understood that the specific compounds set forth above are illustrative and that other compounds containing an alkyl substituent attached to the imino nitrogen and also those containing this substituent and alkyl substituents attached to one or more of the amino nitrogens may be employed.

In another embodiment, the amino or alkylaminotetrahydrocarbazoles may be employed. Illustrative examples of compounds in this class include 6-propylamino-1,2,3,4-tetrahydrocarbazole, 6-butylamino-1,2,3,4-tetrahydrocarbazole, 6-amylamino-1,2,3,4-tetrahydrocarbazole, 6-hexylamino-1,2,3,4-tetrahydrocarbazole, etc.

While the alkyl-substituted amino or polyaminocarbazoles are preferred, it is understood that substituted amino

or polyamino carbazoles in which the substituent comprises other groups may be employed. The other groups preferably comprise hydrocarbon groups and will be selected from cycloalkyl, aryl, alkaryl or aralkyl. In some cases, the substituent may comprise an alkenyl or cycloalkenyl group. In still other cases, the alkyl or other hydrocarbon group may contain non-hydrocarbon components including those comprising oxygen, nitrogen and/or sulfur.

It is understood that mixtures of compounds may be employed. In fact, during the preparation of some of these compounds, a mixture containing two different alkylamino or polyalkylamino compounds is formed, and such mixture may be used.

It is apparent that numerous compounds may be prepared and utilized in accordance with the present invention. However, all of these compounds are not necessarily equivalent and may be of different effectiveness in the same or different greases. The particular compound to be used will depend upon the specific grease to be inhibited and also upon the cost and availability of the inhibitor or of the reactants utilized in the preparation thereof.

In view of an apparent discrepancy in the literature as to the numbering of carbazole compounds, the structural formula of a representative inhibitor compound of the present invention is set forth below to illustrate the numbering system used in the present specification and claims.



The particular carbazole compound illustrated is a 3-alkylaminocarbazole. Again, it is understood that this formula is merely for illustrative purposes and that other suitable alkylamino, including poly-substituted compounds, may be employed.

The inhibitor compounds of the present invention may be prepared in any suitable manner. For example, aminecarbazole may be prepared by nitration of carbazole to form the nitro-substituted compound, followed by reduction of the nitro group to the amino group and by reductive alkylation to form the alkylaminocarbazole. The alkyl substitution preferably is of secondary configuration; that is, the alkyl group is attached to the nitrogen atom at an intermediate carbon atom of the alkyl group. This substitution is obtained by utilizing a ketone in the reductive alkylation reaction. When a primary group is desired, an aldehyde is used in the reductive alkylation step.

In general the inhibitor of the present invention is utilized in a concentration of from about 0.0001% to about 5% by weight of the grease. The exact concentration to be used will depend upon the particular grease being treated. In most cases concentrations of from about 0.01% to about 3% by weight generally is employed.

It is understood that the inhibitor may be used along with other additives incorporated in synthetic grease, including alcohols, esters, organic amines, polybutene, sulfurized fatty materials, sulfur chlorine compounds, dyes, perfumed materials, fillers, etc. In some cases, it may be of advantage to also include a metal deactivator as, for example, disalicylal diamino propane, ethylene diamine tetraacetic acid tetrasodium salt, etc., or to include other additives such as tricresyl phosphate, trialkyl phenols including 2,6-di-tert-butyl-4-methylphenol, 2,4-di-methyl-6-tert-butylphenol, etc., alkylated diphenyl amines, phenyl naphthyl amines, dialkyl phenylene diamines, phenothiazine, organic selenium compounds, etc.,

as well as corrosion inhibitors, extreme pressure additives, viscosity index improvers, etc. The inhibitor of the present invention may be utilized as such or in a suitable solvent including hydrocarbons, alcohols, glycols, ketones, ethers, etc. When desired, the inhibitor may be prepared as a mixture with one or more of these other additives and incorporated in this manner in the grease or components thereof.

The inhibitor of the present invention may be incorporated in the grease in any suitable manner and at any suitable stage of preparation. Thus, it may be added to one or more components of the grease prior to compositing and processing thereof or it may be added to the mix at any time, preferably before final processing in order to obtain intimate mixing and dissolving of the inhibitor in the grease.

The following examples are introduced to illustrate further the novelty and utility of the present invention but not with the intention of unduly limiting the same.

#### Example I

The additive used in this example was 3-octylaminocarbazole and was utilized for the stabilization of a lithium grease commercially available in the open market. The stability of the grease was tested according to a modified Norma-Hoffman method, in which a sample of the grease is placed in a bomb and oxygen is charged thereto. The bomb then is heated to 212° F., and the time required for a drop of 5 pounds' pressure is taken as the induction period. In this run, a control sample of the grease (not containing this additive) had an induction period of 10 hours. On the other hand, a sample of the grease containing 1% by weight of 3-octylaminocarbazole had an induction period of 31 hours. Thus, it is seen that the inhibitor of the present invention served to improve considerably the stability of the grease.

#### Example II

The run described in Example I was continued until a pressure drop of 30 pounds per square inch was obtained. In the control sample, this drop occurred after 23 hours. However, the sample containing 3-octylaminocarbazole ran for 122 hours before reaching the 30 pound pressure drop.

#### Example III

The inhibitor of this example is 3-isopropylaminocarbazole. This compound has a melting point of 181°-182° C. and a boiling point of 170°-190° C. at 1 mm. pressure. This additive is incorporated in a calcium base grease in a concentration of 0.5% by weight and serves to increase the time required for a drop of five pounds pressure when the grease is evaluated in the modified Norma-Hoffman method described in Example I.

#### Example IV

The inhibitor of this example is 3,6-diisopropylaminocarbazole, which compound has a boiling point of 170°-230° C. at 1 mm. pressure. 1.5% by weight of this inhibitor is incorporated in sodium base grease and serves to increase the time required for a drop of 5 pounds' pressure when the grease is evaluated in the modified Norma-Hoffman method described in Example I.

#### Example V

The inhibitor of this example is 1-(2-octylaminocarbazole) and is incorporated in barium base grease in a concentration of 1% by weight. When evaluated in the modified Norma-Hoffman method, the time to reach a drop of 5 pounds' pressure is considerably longer than required in a sample of the grease not containing an inhibitor.

I claim as my invention:

1. A lubricating grease composition consisting essentially of a major amount of a lubricating oil, a grease-

thickening amount of a metal soap of a higher fatty acid and a stabilizing concentration of an alkylaminocarbazole inhibitor.

2. A lubricating grease composition consisting essentially of a major amount of a lubricating oil, a grease-thickening amount of a metal soap of a higher fatty acid and a stabilizing concentration of a polyalkylaminocarbazole inhibitor.

3. A lubricating grease composition consisting essentially of a major amount of a lubricating oil, a grease-thickening amount of a lithium soap of a higher fatty acid and a stabilizing concentration of an alkylaminocarbazole inhibitor.

4. A lubricating grease composition consisting essentially of a major amount of a lubricating oil, a grease-thickening amount of a lithium soap of a higher fatty acid and a stabilizing concentration of a polyalkylaminocarbazole inhibitor.

5. A lubricating grease composition consisting essentially of a major amount of a lubricating oil, a grease-thickening amount of a lithium soap of a higher fatty acid and a stabilizing concentration of 1-(2-octylaminocarbazole).

6. A lubricating grease composition consisting essentially of a major amount of a lubricating oil, a grease-thickening amount of a lithium soap of a higher fatty acid and a stabilizing concentration of 3-octylaminocarbazole.

7. A lubricating grease composition consisting essentially of a major amount of a lubricating oil, a grease-thickening amount of a lithium soap of a higher fatty acid and a stabilizing concentration of 3-isopropylaminocarbazole.

8. A lubricating grease composition consisting essen-

tially of a major amount of a lubricating oil, a grease-thickening amount of a lithium soap of a higher fatty acid and a stabilizing concentration of 3,6-diisopropylaminocarbazole.

9. A lubricating grease composition consisting essentially of a major amount of a lubricating oil, a grease-thickening amount of a calcium soap of a higher fatty acid and a stabilizing concentration of 3-octylaminocarbazole.

10. A lubricating grease composition consisting essentially of a major amount of a lubricating oil, a grease-thickening amount of a calcium soap of a higher fatty acid and a stabilizing concentration of 3-isopropylaminocarbazole.

11. A lubricating grease composition consisting essentially of a major amount of a lubricating oil, a grease-thickening amount of lithium stearate and from about 0.0001% to about 5% by weight of an alkylaminocarbazole inhibitor.

12. A lubricating grease composition consisting essentially of a major amount of a lubricating oil, a grease-thickening amount of calcium stearate and from about 0.0001% to about 5% by weight of an alkylaminocarbazole inhibitor.

#### References Cited in the file of this patent

#### UNITED STATES PATENTS

|           |                |       |                |
|-----------|----------------|-------|----------------|
| 1,836,702 | Christmann     | ----- | Dec. 15, 1931  |
| 2,370,552 | Lincoln et al. | ----- | Feb. 27, 1945  |
| 2,374,098 | Ingram         | ----- | Apr. 17, 1945  |
| 2,595,140 | Heinrich       | ----- | Apr. 29, 1952  |
| 2,607,735 | Sproule et al. | ----- | Aug. 19, 1952  |
| 2,652,366 | Jones et al.   | ----- | Sept. 15, 1953 |